# EUROPEAN PATENT SPECIFICATION

(11) **EP 0 990 069 B1**
(45) Date of publication and mention of the grant of the patent: **22.08.2001**
(21) Application number: 98919272.9
(22) Date of filing: 08.04.1998
(51) Int. Cl.: D21F 9/00

(54) **PROCESS AND PLANT FOR PAPER AND PAPERBOARD PRODUCTION STARTING FROM WASTE PAPER**
VERFAHREN UND VORRICHTUNG ZUR HERSTELLUNG VON PAPIER UND PAPPE AUS ALTPAPIER
PROCEDE ET INSTALLATION DE PRODUCTION DE PAPIER ET DE CARTON A PARTIR DE VIEUX PAPIERS

(30) Priority: 18.04.1997 IT MI970904
(43) Date of publication of application: 05.04.2000
(73) Proprietor: Locati, Giuseppe, 20052 Monza (Milano) (IT)
(72) Inventor: Locati, Giuseppe, 20052 Monza (Milano) (IT)
(74) Representative: Faraggiana, Vittorio, Dr. Ing.
(86) International application number: EP9802215
(87) International publication number: WO9848110

(56) References cited:
- WO-A-95/12020
- GB-A- 1 372 502
- US-A- 2 746 895
- US-A- 3 718 536
- US-A- 3 949 035

## Description

The present invention relates to a process 'and a plant for paper and paperboard production. In particular, the invention relates to a continuous-flow production, with a minimum use of water and energy, starting from waste paper.

It is known that in paper production employment of great amounts of water is required. Usually, the adopted process comprises a paper maceration step carried out in plenty of water, so as to separate the long natural fibres. These fibres are subsequently coupled with each other by drop and light compression between cloths and felts. Finally, the product thus obtained is submitted to a drying step.

In addition to the high amount of water required, there is therefore also a great waste of energy due both to the necessity of removing water from the product, and the necessity of a long treatment step of the polluted water thus produced.

WO 95/12020 discloses a process for the production of a fibrous sheet material by means of dry-laying cellulosic fibres on a continuously moving support to form a layer thereon and wetting the layer sufficiently to cause hydrogen bonds to be formed. However, the product obtained by this method needs further processing to be utilizable.

It is a general object of the present invention to obviate the above mentioned drawbacks by providing a process and a plant for paper production starting from waste paper, with a low water amount, preferably without production of impregnation water to be evacuated and a limited waste of energy.

In view of this object, in accordance with the invention a process for paper or paperboard production has been devised which comprises the steps of:
- chopping up waste paper to reduce it to particles;
- laying down particles into an even layer to form a mat;
- spraying the mat with water;
- submitting the mat to a compression of at least 19,6 MPa (200kg/cm²) and preferably between 29,4 and 49 MPa (between 300 and 500kg/cm²).

In accordance with this process also provided is a plant for paper or paperboard production, comprising:
- means for chopping up waste paper until it is reduced to particles;
- first distribution means to lay down particles into an even layer to form a mat;
- spraying means for spraying the mat with water;
- pressing means to submit the mat to a compression of at least 19,6 MPa (200kg/cm²) and preferably between 29,4 and 49 MPa (between 300 and 500kg/cm²).

For better explaining the innovatory principles of the present invention and the advantages it offers over the known art, a possible embodiment applying said principles will be given hereinafter, by way of non-limiting example, with reference to the accompanying sole drawing.

With reference to the figure, a plant 10 for paper production in accordance with the invention is diagrammatically shown.

The plant is comprised of a device 11 for producing paper fragments or powder that are sent to a first distributor 12 to form a layer 13 on a belt conveyor 14. Fragments can be advantageously reduced to average sizes not exceeding 7mm and, preferably, comprised between 2mm and 5mm. A spraying device 15 wets, advantageously by shower atomization, the layer formed on the mat so as to produce a damp mat or ribbon. A second distributor 16 may be provided for distributing a second layer of paper fragments or powder on the first damp layer. Thus a mat or ribbon is obtained which is formed of two layers of paper fragments with a water film between the two layers.

The damp paper-fragment ribbon is passed into a pressing device 17 and a compact ribbon 18 comes out of it. Pressing takes place at pressures at least as high as 19,6 MPa (200kg/cm²) and, preferably, between 29,4 and 49 MPa (between 300 and 500kg/cm²). Advantageously, the amount of water distributed over the fragment layer is selected in such a manner that pressing does not produce an important water extraction from the paper ribbon. For example, it has been found advantageous for the water amount to be lower than or equal to one litre per paper kg. By virtue of pressing, the sprayed water which is between the layers is forced to penetrate at least partly into the layers and the paper ribbon dampness is thus substantially made uniform in the ribbon thickness. The outgoing ribbon is just slightly damp.

It has been noted that the paper ribbon thus obtained has an excellent cohesion, comparable with that obtained with paper produced following traditional methods, although made of paper fragments.

The ribbon thus obtained can be submitted to a further pressing operation by means of rollers 19, for providing a further surface finish, for example. If the residual retained water amount is considered still too much, the paper ribbon may be further submitted to a drying step 20. Once the paper production steps have been completed, paper can be wound onto a bobbin 21.

Distribution of paper fragments to form the two layers on the mat can be accomplished by means of inclined vibration screens 22, 24 having appropriate mesh sizes based on the desired fragment sizes. Possible fragments of bigger sizes can be gathered into containers 23, 24 at the lower screen end to be then recirculated and sent to the chopping device 11 again.

The chopping or mincing device 11 can be formed of a toothed rotary drum 26 against which the waste paper mass 27 is pushed by means of a press 28.

The minced paper particles can be assimilated to flocks; therefore they are quite different from cellulose fibres of greater or smaller length that are usually necessary in paper production according to the known art.

The paper particles before reaching distributors 12, 16 can also be mixed in a mixer 29 with other particles of different production. For instance, colour of the produced paper can be adjusted by mixing particles produced from chopping of paper particles of different composition and source.

The paper ribbon pressing and squeezing device 17 can advantageously consist of the end portion of conveyor 14 and a rotary belt 30 disposed to have a stretch facing said end portion of the conveyor belt 14. Belts 14 and 30 are driven in movement at the same speed and the faced stretches are pushed against each other by pressing rollers 31, 32 disposed face-to-face on opposite belt faces.

The belt material is such selected as to be pervious to water or in any case capable of enabling removal of water from the ribbon which is squeezed between the belts.

At this point it is apparent that the intended purposes have been reached.

Water supply can be of the strictly necessary amount for a correct damping of layers. Pressing causes the water to pass through the layers from inside to outside reaching a perfect layer permeation. The residual dampness is very low and, should it be necessary, can be easily removed by quick drying with a low energy consumption. By adjusting the sprayed water amount, there is practically no water to be drawn.

Thus, high water consumption does not exist and water purification operations which are peculiar to the known art are not required.

The plant in accordance with the invention is very simple and manufacture and servicing of same is easy and cheap. Production of two or more layers enables manufacture of paper and paperboard having different surface features on the two faces to be carried out. A process in accordance with the invention is adapted to make simple or two-faced paper or paperboards consisting either of a single layer or of superposed layers.

Thickness of the produced layers can be easily varied and checked by masking the perforated surfaces of the vibration screens, for example.

Unlike the known art, the plant can be easily and readily stopped and re-started, in order to comply, for instance, with work shifts, ordinary and extraordinary maintenance requirements, production controls or changes, etc. Obviously, the above description of an embodiment applying the innovatory principles of the present invention is reproduced by way of example only and cannot be considered as a limitation of the inventive scope as herein claimed. For example, should it be necessary, additives may be added to the atomized water for meeting particular requirements, the additive amounts being substantially those that are strictly necessary for the produced amount of paper, without wastes and without recovery being required. A small amount of glue or paste can be optionally added to water. For instance, it has been found that with more than 20% of glue in the water a nearly coated thin paperboard can be obtained.

## Claims

1. A process for paper or paperboard production comprising the steps of:
- chopping up waste paper to reduce it to particles;
- laying down particles into an even layer to form a mat;
- spraying the mat with water;
- submitting the mat to a compression of at least 19,6 MPa (200kg/cm²) and preferably between 29,4 and 49 MPa (between 300 and 500kg/cm²).

2. A process as claimed in claim 1, comprising the further step of laying down a second particle layer on the first layer after the spraying step and before the pressing step.

3. A process as claimed in claim 1, characterized in that spraying is carried out by shower atomization.

4. A process as claimed in claim 1, characterized in that compression is carried out by pressing rollers while the mat is being passed between facing conveyor belts.

5. A process as claimed in claim 1, comprising a further pressing step downstream of the first pressing step.

6. A process as claimed in claim 1, comprising the further step of decreasing the water content in the mat by heating.

7. A process as claimed in claim 1, in which there is such a water supply that substantially no water drawing from the mat occurs during the compression step.

8. A process as claimed in claim 1, in which water supply is lower than or almost equal to one litre per paper kg.

9. A process as claimed in claim 1, in which particles have an average size not exceeding 7mm and, preferably, included between 2mm and 5mm.

10. A plant for paper or paperboard production, comprising:
- means (11) for chopping up waste paper until it is reduced to particles;
- first distribution means (12) to lay down particles into a uniform layer to form a particle mat;
- spraying means (15) for spraying the mat with water;
- pressing means (17) to submit the mat to a compression of at least 19,6 MPa (200kg/cm²) and preferably between 29,4 and 49 MPa (between 300 and 500kg/cm²).

11. A plant as claimed in claim 10, characterized in that it comprises second distribution means (16) to lay down a second particle layer on the first layer, which means is disposed between the spraying means (15) and the pressing means (17).

12. A plant as claimed in claim 10, characterized in that the spraying means (15) carries out shower atomization onto the layer.

13. A plant as claimed in claim 10, characterized in that the pressing means (17) comprises facing pressing rollers (31, 32) between faced stretches of conveyor belts (14, 30) between which the particle mat runs.

14. A plant as claimed in claim 10, characterized in that the particle mat is formed on a conveyor belt (14) passing close to the different distribution, spraying and pressing means.

15. A plant as claimed in claim 10, characterized in that it comprises further mat pressing means (19) disposed downstream of the first pressing means.

16. A plant as claimed in claim 10, characterized in that it comprises drying means (20) to decrease the water content in the mat downstream of the pressing means.

17. A plant as claimed in claim 11, characterized in that the distribution means (12, 16) comprises vibration screens (22, 24).

18. A plant as claimed in claim 10, characterized in that the paper chopping means (11) comprises a toothed rotary drum (26) against which the waste paper mass (27) is forced.

19. A plant as claimed in claim 10, characterized in that at the outlet of the paper chopping means (11), particles have an average size not exceeding 7mm and preferably included between 2mm and 5mm.

20. A process according to claim 1, characterized in that it comprises the further step of laying down a second layer of chopped waste paper particles on the first layer after the spraying step and before the pressing step to form a mat consisting of two layers of chopped waste paper particles with a water film therebetween, the compression step forcing the water to the outside through the layers.

## Patentansprüche

1. Verfahren zur Herstellung von Papier oder Pappe, umfassend die Schritte:
- Zerkleinern von Altpapier, um es zu Partikeln zu reduzieren;
- Ablegen der Partikel in einer gleichmäßigen Lage, um eine Matte zu bilden;
- Besprühen der Matte mit Wasser;
- Komprimieren der Matte mit wenigstens 19,6 MPa (200 kg/cm²) und vorzugsweise zwischen 29,4 und 49 MPa (zwischen 300 und 500 kg/cm²).

2. Verfahren nach Anspruch 1, umfassend den weiteren Schritt, dass eine zweite Partikellage auf der ersten Lage nach dem Besprühschritt und vor dem Pressschritt abgelegt wird.

3. Verfahren nach Anspruch 1, dadurch gekennzeichnet, dass das Besprühen durch Duschzerstäubung durchgeführt wird.

4. Verfahren nach Anspruch 1, dadurch gekennzeichnet, dass die Kompression durch Druckwalzen ausgeführt wird, während die Matte zwischen einander zugewandten Förderbändern hindurchgegeben wird.

5. Verfahren nach Anspruch 1, umfassend einen weiteren Preßschritt stromab von dem ersten Preßschritt.

6. Verfahren nach Anspruch 1, umfassend den weiteren Schritt, dass der Wassergehalt in der Matte durch Heizen herabgesetzt wird.

7. Verfahren nach Anspruch 1, bei dem eine solche Wasserzufuhr vorhanden ist, dass im wesentlichen kein Wasserabzug aus der Matte während des Kompressionschrittes stattfindet.

8. Verfahren nach Anspruch 1, bei dem die Wasserzufuhr geringer als oder nahezu gleich einem Liter pro kg Papier ist.

9. Verfahren nach Anspruch 1, bei dem die Partikel eine mittlere Größe von nicht mehr als 7 mm und vorzugsweise zwischen 2 mm und 5 mm haben.

10. Anlage zur Herstellung von Papier oder Pappe, umfassend:
- eine Einrichtung (11) zum Zerkleinern von Altpapier, bis es zu Partikeln reduziert ist;
- eine erste Verteilereinrichtung (12), um die Partikel in einer gleichmäßigen Lage abzulegen, um eine Partikelmatte zu bilden;
- eine Sprüheinrichtung (15) zum Besprühen der Matte mit Wasser;
- eine Presseinrichtung (17), um die Matte einer Kompression von wenigstens 19,6 MPa (200 kg/cm²) und vorzugsweise zwischen 29,4 und 49 MPa (zwischen 300 und 500 kg/cm²) zu unterwerfen.

11. Anlage nach Anspruch 10, dadurch gekennzeichnet, dass sie eine zweite Verteilereinrichtung (16) umfasst, um eine zweite Partikellage auf der ersten Partikellage abzulegen, wobei die Einrichtung zwischen der Sprüheinrichtung (15) und der Presseinrichtung (17) liegt.

12. Anlage nach Anspruch 10, dadurch gekennzeichnet, dass die Sprüheinrichtung (15) eine Duschzersteubung auf die Lage ausführt.

13. Analge nach Anspruch 10, dadurch gekennzeichnet, dass die Presseinrichtung (17) einander gegenüberliegende Druckwalzen (31, 32) zwischen einander zugewandten Strecken von Förderbändern (14; 30) aufweist, zwischen denen die Partikelmatte läuft.

14. Analge nach Anspruch 10, dadurch gekennzeichnet, dass die Partikelmatte auf einem Förderband (14) gebildet ist, das nahe an den verschiedenen Verteiler-, Sprüh- und Presseinrichtungen vorbeiläuft.

15. Analge nach Anspruch 10, dadurch gekennzeichnet, dass sie eine weitere Matten-Presseinrichtung (19) umfasst, die stromab von der ersten Presseinrichtung angeordnet ist.

16. Analge nach Anspruch 10, dadurch gekennzeichnet, dass sie eine Trockeneinrichtung (20) umfasst, um den Wassergehalt in der Matte stromab von der Presseinrichtung zu verringern.

17. Analge nach Anspruch 11, dadurch gekennzeichnet, dass die Verteilereinrichtungen (12, 16) Vibrationssiebe (22, 24) umfasst.

18. Analge nach Anspruch 10, dadurch gekennzeichnet, dass die Papierzerkleinerungseinrichtung (11) eine gezahnte, rotierende Trommel (26) umfasst, gegen die die Altpapiermasse (27) gedrückt wird.

19. Analge nach Anspruch 10, dadurch gekennzeichnet, dass an dem Auslass der Papierzerkleinerungseinrichtung (11) Partikel mit einer mittleren Größe von nicht mehr als 7 mm und vorzugsweise zwischen 2 mm und 5 mm vorhanden sind.

20. Verfahren nach Anspruch 1, dadurch gekennzeichnet, dass es den weiteren Schritt umfasst, dass eine zweite Schicht von zerkleinerten Altpapierpartikeln auf der ersten Lage nach dem Sprühschritt und vor dem Pressschritt abgelegt wird, um eine Matte zu bilden, die aus zwei Lagen von zerkleinerten Altpapierpartikeln mit einem Wasserfilm dazwischen gebildet wird, wobei der Kompressionsschritt das Wasser durch die Schichten nach außen drückt.

## Revendications

1. Procédé de production de papier ou carton comprenant les étapes consistant à:
- hacher des vieux papiers pour les réduire à l'état de particules;
- déposer les particules sous la forme d'une couche uniforme de manière à former un mat;
- pulvériser de l'eau sur le mat;
- soumettre le mat à une compression égale à au moins 19,6 MPa (200 kg/cm²) et de préférence entre 29,4 et 49 MPa (entre 300 et 500 kg/cm²).

2. Procédé selon la revendication 1, comprenant l'étape supplémentaire consistant à disposer une seconde couche de particules sur la première couche après l'étape de pulvérisation et avant l'étape de compression.

3. Procédé selon la revendication 1, caractérisé en ce que la pulvérisation est effectuée par une atomisation du type semblable à celle fournie par une douche.

4. Procédé selon la revendication 1, caractérisé en ce que la compression est exécutée par des rouleaux de pressage, tandis que le mat passe entre des bandes convoyeuses situées en vis-à-vis.

5. Procédé selon la revendication 1, comprenant une autre étape de pressage en aval de la première étape de pressage.

6. Procédé selon la revendication 1, comprenant l'étape supplémentaire de réduction, par chauffage, de la teneur en eau dans le mat.

7. Procédé selon la revendication 1, dans lequel il existe une alimentation en eau telle que pour l'essentiel aucun soutirage d'eau du mat ne se produit pendant l'étape de compression.

8. Procédé selon la revendication 1, selon lequel l'alimentation en eau est inférieure ou presque égale à un litre par kg de papier.

9. Procédé selon la revendication 1, selon lequel les particules possèdent une taille moyenne ne dépassant pas 7 mm et de préférence comprise entre 2 mm et 5 mm.

10. Installation pour la production de papier ou de carton, comprenant:
- des moyens (11) pour hacher des vieux papiers jusqu'à ce qu'ils soient réduits à l'état de particules;
- des premiers moyens de distribution (12) pour déposer des particules sous la forme d'une couche uniforme de manière à former un mat de particules;
- des moyens de pulvérisation (15) pour pulvériser de l'eau sur le mat;
- des moyens de pressage (17) pour soumettre le mat à une compression égale à au moins 19,6 MPa (200 kg/cm²) et de préférence comprise entre 29,4 et 49 MPa (entre 300 et 500 kg/cm²).

11. Installation selon la revendication 10, caractérisée en ce qu'elle comprend des seconds moyens de distribution (16) pour déposer une seconde couche de particules sur la première couche, lesquels moyens sont disposés entre les moyens de pulvérisation (15) et les moyens de pressage (17).

12. Installation selon la revendication 10, caractérisée en ce que les moyens de pulvérisation (15) exécutent une atomisation à la manière d'une douche sur la couche.

13. Installation selon la revendication 10, caractérisée en ce que les moyens de pressage (17) comprennent des rouleaux de pressage (31, 32), qui se font face, entre des brins, situés en vis-à-vis, de bandes convoyeuses (14, 30) entre lesquelles circule le mat de particules.

14. Installation selon la revendication 10, caractérisée en ce que le mat de particules est formé sur une bande convoyeuse (14) qui passe à proximité des différents moyens de distribution, de pulvérisation et de pressage.

15. Installation selon la revendication 10, caractérisée en ce qu'elle comprend en outre des moyens supplémentaires (19) de pressage du mat disposés en aval des premiers moyens de pressage.

16. Installation selon la revendication 10, caractérisée en ce qu'elle comprend des moyens de séchage (2.0) pour réduire la teneur en eau dans le mat en aval des moyens de pressage.

17. Installation selon la revendication 11, caractérisée en ce que les moyens de distribution (12, 16) comprennent des tamis vibrants (22, 24).

18. Installation selon la revendication 10, caractérisée en ce que les moyens (11) de hachage du papier comprennent deux tambours dentés rotatifs (26), contre lesquels la masse de vieux papiers (27) est repoussée.

19. Installation selon la revendication 10, caractérisée en ce qu'à la sortie des moyens (11) de hachage du papier, les particules possèdent une taille moyenne ne dépassant pas 7 mm et comprise de préférence entre 2 mm et 5 mm.

20. Procédé selon la revendication 1, caractérisé en ce qu'il comprend l'étape supplémentaire consistant à déposer une seconde couche de particules de vieux papiers hachés sur la première couche après l'étape de pulvérisation et avant l'étape de pressage pour former un mat constitué de deux couches de particules de vieux papiers hachés, entre lesquelles est intercalé un film d'eau, l'étape de compression refoulant l'eau à force vers l'extérieur à travers les couches.
